

## UNITED STATES PATENT OFFICE

2,664,354

## VALVES FOR INTERNAL COMBUSTION ENGINES

Clarence George Bieber and Walter Franklin Sumpter, Huntington, W. Va., assignors to The International Nickel Company, Inc., New York, N. Y., a corporation of Delaware

No Drawing. Application October 12, 1950,  
Serial No. 189,894

## 4 Claims. (Cl. 75—171)

**1** The present invention relates to special heat-resisting articles, such as valves, valve seats, valve stems, and other structural components of internal combustion engines which are subjected in use at elevated temperatures to destructive actions, particularly the corrosive action of oxidizing, neutral, and reducing atmospheres containing substantial amounts of combusted lead-containing fuels, and to special heat-resisting, silicon-containing, nickel-chromium alloys for such articles.

It is well known in the art that alloys employed as valves or valve parts in internal combustion engines must possess resistance to creep and resistance to corrosion, erosion, and pitting at elevated temperatures and must also be able to resist various destructive influences under operating conditions. This is particularly true of structural components of internal combustion engines in which leaded gasolines are employed as fuel. The combustion products of leaded gasolines contain very corrosive materials, such as lead, lead oxide, lead sulfide, lead sulfate, and other lead compounds, e. g. lead bromide, which are extremely destructive to valve alloys in that these lead-containing combustion products cause premature failure of valves, valve parts, etc., due to corrosion, erosion, and pitting, especially under conditions involving fluctuating lead-containing atmospheres, i. e., varying from oxidizing to neutral to reducing conditions and/or vice versa. Ordinarily, valves employed in service are subjected in the main to oxidizing conditions. However, under conditions involving full power operation, such as exist in airplanes during take-off and rapid climb, valves are subjected to reducing conditions which detrimentally affect the life of the valve alloy. By "reducing conditions" is meant an atmosphere which is reducing to lead oxide or other lead compounds contained in combusted fuels of internal combustion engines as exemplified by a combusted lead-containing atmosphere containing an excess of carbon monoxide or hydrogen in amounts reducing to lead oxide or other lead compounds. Certain silicon-containing alloys have been used for valves but have been found only partially effective. While some of these silicon-containing alloys show fairly good corrosion resistance in oxidizing lead-containing atmospheres, these silicon-containing alloys did not always stand up in reducing lead-containing atmospheres. One attempt made to alleviate the burden placed upon valves subjected to fluctuating atmospheres of combusted lead-containing fuels in internal combustion en-

**2** gines involved the introduction of sodium-cooled, hollow head valves with the aim of improving valve life by preventing over-heating of valves while in service. Another attempt involved the use of the "positive valve rotator" to insure proper valve seating, to maintain efficiency of valve operation, and to improve valve life. Still another attempt made to improve the over-all resistance of valves to corrosion by fluctuating atmospheres of combusted lead-containing fuels involved the hard facing of valves with special corrosion resistant alloys, e. g., carbon-containing, non-ferrous alloys of the cobalt-chromium-tungsten type. While the foregoing attempts have been partially beneficial in prolonging valve life, continual demands by industry for more powerful and for higher speed engines have placed further burdens on valve alloys with the result that the valve problem, including valve corrosion, valve erosion, and valve pitting, has become accentuated.

Although many attempts were made to meet the needs of industry and to overcome the foregoing difficulties and disadvantages, none, as far as we are aware, was entirely successful when carried into practice commercially on an industrial scale.

It has now been discovered that the problem confronting the art of providing corrosion-resistant, silicon-containing, valve alloys for use at elevated temperatures in internal combustion engines employing corrosive lead-containing fuels can be overcome by utilizing a heat-treated, silicon-containing, nickel-chromium alloy containing a novel combination of elements within critical ranges.

It is the object of the present invention to provide an improved heat-treatable, silicon-containing valve alloy which has resistance to creep, combined with resistance to corrosion, erosion, and pitting when used in internal combustion engines.

Another object of the invention is to provide an improved heat-treatable, silicon-containing alloy for use as valves or valve parts in internal combustion engines in which leaded gasoline fuel is employed.

The invention also contemplates providing a heat-treatable alloy for valves and valve parts in internal combustion engines with the purpose of improving performance characteristics of internal combustion engines and extending valve life.

It is the further object of the invention to provide a special heat-resisting, silicon-containing,

nickel-base alloy for use as component material in internal combustion engines, said alloy being heat-treatable and having improved corrosion resistance when exposed to fluctuating atmospheres containing lead, lead oxide, lead sulfide, lead sulfate, and other lead compounds, e. g., lead bromide.

It is also the object of the invention to provide a heat-treated valve part having improved resistance to corrosion, erosion, and pitting when exposed to lead-containing combustion gases under reducing conditions and made of the silicon-containing, nickel-base alloy provided by the present invention.

Other objects and advantages will become apparent from the following description.

Generally speaking, the present invention provides valve parts for internal combustion engines comprised of a heat-treatable, silicon-containing, nickel-chromium alloy containing critical amounts of titanium, silicon, manganese, and iron. The valve parts made at least in part of the present heat-treatable alloys, when exposed to the corrosive action of fluctuating atmospheres of lead-containing gases at elevated temperatures, i. e., gaseous combustion products of leaded fuels such as commonly prevail in internal combustion engines, exhibit an improved combination of chemical and physical properties, such as resistance to corrosion, erosion, and pitting, combined with excellent creep resistance and excellent strength and toughness at elevated temperatures, which combination of properties heretofore was not exhibited by valve parts made of prior art alloys.

More particularly, the present invention provides a valve part for internal combustion engines, e. g., a valve, comprised of a heat-treatable, silicon-containing, nickel-base alloy in which the silicon content is critically controlled in the presence of titanium, manganese, and iron. The broad composition range of the heat-treatable, nickel-base alloy which has been found to give the results desired when employed as a valve alloy comprises about 15% to 17% chromium, up to about 8% iron, about 0.05% to 2.5% manganese, about 2.75% to 3.35% titanium, up to about 0.15% silicon, and the balance substantially all nickel. In employing the foregoing alloy in valve and valve parts of internal combustion engines, it is preferred that the manganese content should not be less than 1.75%. In addition, the alloy is preferably made substantially devoid of aluminum and carbon, although up to about 0.10% aluminum and up to about 0.10% carbon may be tolerated in the alloy without deleteriously affecting the alloy. The alloy may also contain small amounts of the incidental elements, such as copper, etc. Impurities, such as sulfur, lead, selenium, tellurium, bismuth, etc., are kept as low as is commercially practicable.

In carrying the invention into practice, it is preferred to have the valve alloy contain about 15% to 17% chromium, about 3% to 8% iron, about 2% to 2.5% manganese, about 2.85% to 3.35% titanium, about 0.005% to 0.10% silicon, and the balance substantially all nickel. As nickel usually contains a small amount of cobalt in association therewith, it is understood that the term "nickel" as employed herein includes cobalt in incidental amounts, e. g., up to about 1%. Titanium, which is essential as an age-hardening strengthener, is maintained at least as high as about 2.75% and is preferably held at about 2.85% or higher in applications involving structural components of heavy-duty internal com-

bustion engines in which high physical strength and high hot hardness are important. Under conditions where optimum age hardening effect of titanium is desired, the carbon content of the alloy is kept as low as is commercially practicable and preferably does not exceed 0.03% maximum. As stated hereinbefore, the alloy is substantially devoid of aluminum which does not exceed about 0.10% of the alloy composition.

In testing alloys for their valve properties, hot hardness and the lead oxide corrosion, laboratory tests are often employed. The lead oxide test, which is used to confirm good properties of valve alloys, i. e., resistance of valve alloys to corrosion by lead-containing compounds, comprises testing a sample of the alloy in contact with molten lead oxide for a given length of time at a temperature of about 1650° F. under reducing conditions. While oxidizing conditions have been heretofore employed to test valve alloys in molten lead oxide, the resistance of valve alloys to lead oxide corrosion under oxidizing conditions is not the only criterion. Thus, alloys which showed excellent resistance to corrosion under oxidizing conditions were not always satisfactory and in many instances were bad when employed as valves.

Several examples of alloys within the scope of the invention were tested for corrosion resistance in molten lead oxide and were found to have good properties. In testing these alloys, the specimens were solution treated for two hours at 2000° F. and then subjected to the destructive action of molten lead oxide for a given length of time at a temperature of about 1650° F. in a reducing combusted natural gas atmosphere containing about 6% carbon monoxide. Two alloys, which showed excellent valve properties when subjected to the lead oxide test, are given in Table I as follows:

Table I

| Alloy No. | Percent Ni | Percent Cr | Percent Ti | Percent Fe | Percent Si | Percent Mn | Percent C |
|-----------|------------|------------|------------|------------|------------|------------|-----------|
| 1         | 78.62      | 15.81      | 3.07       | 0.33       | 0.12       | 1.92       | 0.07      |
| 2         | 78.32      | 15.64      | 2.96       | 5.97       | 0.07       | 1.93       | 0.06      |

Alloy No. 1 and alloy No. 2 gave excellent results on the weight loss basis insofar as overall corrosion was concerned when exposed to the corrosive action of molten lead oxide in the aforementioned test. Alloy No. 1 and alloy No. 2 also showed a greatly reduced tendency to pitting corrosion.

A series of alloys within the scope of the invention, which were also tested in molten lead oxide under reducing conditions in accordance with the foregoing test procedure, are given in Table II.

Table II

| Alloy No. | Percent Ni | Percent Cr | Percent Ti | Percent Fe | Percent Si | Percent Mn | Percent C | Percent Al |
|-----------|------------|------------|------------|------------|------------|------------|-----------|------------|
| 3         | 77.95      | 15.95      | 2.74       | 2.87       | 0.18       | 0.08       | 0.08      | 0.022      |
| 4         | 78.1       | 15.32      | 2.88       | 0.20       | 0.08       | 0.49       | 0.01      | 0.044      |
| 5         | 72.62      | 15.67      | 2.77       | 6.62       | 0.13       | 2.04       | 0.04      | 0.023      |
| 6         | 72.59      | 15.38      | 2.90       | 6.52       | 0.15       | 2.29       | 0.03      | 0.017      |
| 7         | 72.90      | 15.36      | 2.99       | 6.36       | 0.14       | 2.17       | 0.02      | 0.016      |
| 8         | 72.98      | 15.36      | 2.94       | 6.32       | 0.13       | 2.19       | 0.02      | 0.014      |
| 9         | 73.14      | 15.36      | 2.86       | 6.33       | 0.05       | 2.18       | 0.02      | 0.012      |
| 10        | 73.11      | 15.35      | 2.75       | 6.36       | 0.11       | 2.33       | 0.03      | 0.017      |

Alloys Nos. 1 to 10 illustrate the various compositions of valve alloys which can be employed in internal combustion engines under severe operat-

ing conditions and which resist the corrosive action of combusted lead-containing atmospheres under both oxidizing and reducing conditions.

For the purpose of giving those skilled in the art a better appreciation of the present invention, a series of comparative tests were conducted with alloys having compositions outside the scope of the invention. These alloys were similarly exposed to the corrosive action of lead oxide at a temperature of about 1650° F. in a reducing, combusted, natural-gas atmosphere as hereinbefore described. For convenience, the alloys having compositions outside the scope of the present invention are listed in the following Table III.

Table III

| Alloy | Percent Ni | Percent Cr | Percent Ti | Percent Fe | Percent Si | Percent Mn | Percent C | Percent Al | Percent others |
|-------|------------|------------|------------|------------|------------|------------|-----------|------------|----------------|
| A     | 79.90      | 18.98      |            | 0.35       | 0.35       | 0.32       | 0.02      |            |                |
| B     | 74.74      | 24.12      |            | 0.37       | 0.41       | 0.28       | 0.02      |            |                |
| C     | 71.53      | 19.79      |            | 7.99       | 0.36       | 0.33       | 0.01      |            |                |
| D     | 74.69      | 24.50      |            | 10.09      | 0.29       | 0.34       | 0.03      |            |                |
| E     | 6.62       | 23.65      |            | Bal.       | 0.07       | 0.59       | 0.41      |            | 2.87 Mo        |
| F     | 15.04      | 29.38      |            | Bal.       | 0.05       | 0.12       | 0.50      |            | 14.46 Co       |
| G     | 0.47       | 22.37      |            | Bal.       | 0.14       | 13.44      | 1.28      |            |                |
| H     | 34.40      | 17.70      | 1.83       | Bal.       | 0.12       | 0.22       | 0.08      | 0.02       |                |
| I     | Bal.       | 15.04      | 2.79       | 0.40       | 0.98       |            |           |            |                |
| J     | Bal.       | 15.07      | 2.89       | 17.0       | 0.03       | 2.06       | 0.02      | 0.034      |                |

All of the alloys listed in Table III were unsatisfactory and failed under the aforementioned lead oxide test. Alloys E to J exhibited particularly poor properties as evidenced by very bad overall corrosion and very bad pitting.

The new and improved results provided by the present invention are obtained by subjecting the novel alloys to an appropriate age-hardening heat treatment to impart thereto an age-hardened structure as is well known to those skilled in the art. The heat treatment can comprise a high temperature solution treatment at a temperature within the range of about 1900° F. to about 2100° F., followed by rapid cooling to below about 1500° F. in order to maintain most of the precipitable phases in solid solution, and by a subsequent aging treatment in the temperature range of about 1250° F. to about 1350° F. A preferred age-hardening heat treatment comprises heating at a temperature between about 1960° F. and about 2000° F., rapidly cooling to below about 1300° F. and then aging for about 16 to about 20 hours at about 1300° F. In employing an age-hardening heat treatment on articles made of the alloy, e. g., valves, valve parts, etc., the solution treatment may be conducted as part of the hot working operation and, furthermore, it is not always necessary to use the high temperature solution treatment. Where it is desired to modify the combination of properties, e. g., at elevated operating temperatures, the foregoing heat treatments can be varied. Thus, a treatment above the aging temperature can be employed prior to the aforementioned aging treatment to modify the combination of properties at elevated temperatures. Such an intermediate treatment can be conducted within the range of about 1400° F. to 1750° F., e. g., at about 1400° F., or 1450° F., or 1500° F., or 1550° F., or 1600° F., or 1650° F.

By employing the novel combination of elements within the composition range contemplated by the present invention and heat treating in accordance with the foregoing, the valve alloys provided by the present invention possess high temperature physical and chemical properties markedly superior to those possessed by conventional valve alloys.

In the heat-treated condition, the novel alloys are particularly suitable for use as valves, valve parts, and other structural elements of internal combustion engines, including gas turbines and jet engines. These structural elements can be made entirely of the alloy or partly of the alloy. Thus, the structural elements can be cladded with the alloy.

The present invention is particularly applicable to parts for heavy-duty, internal combustion engines, e. g., valves, valve parts, and other structural elements, and especially applicable for service under extremely corrosive conditions, such as those involving reducing atmospheres as well as oxidizing and neutral atmospheres resulting from the combustion of leaded fuels.

It is to be observed that the present invention provides as an article of manufacture a heat-resistant internal combustion engine valve or valve part having resistance to the destructive action of combusted leaded fuels and comprising an age-hardened, silicon-containing, nickel-base alloy.

Furthermore, the present invention provides a structural element which in normal use is subjected to the destructive action of combusted lead-containing fuels at elevated temperatures in internal combustion engines.

Moreover, the present invention provides a heat-resistant alloy having substantial resistance to the destructive action of corrosive lead-containing atmospheres at elevated temperatures and particularly suitable for valves, valve parts, and other structural elements of internal combustion engines, including gas turbines and jet engines.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A hollow-headed internal combustion engine valve subjected in use at elevated temperatures to the destructive action of fluctuating atmospheres of combusted lead-containing fuels under oxidizing, neutral and reducing conditions, said hollow-headed valve being comprised of an age-hardened, silicon-containing, nickel-base alloy possessing corrosion resistance to the lead oxide test and consisting essentially of about 15% to 17% chromium, about 2.85% to 3.35% titanium, about 2% to 2.5% manganese, about 0.005% to 0.10% silicon, up to about 0.08% carbon, about 3% to 8% iron, and the balance essentially nickel, said alloy being devoid of aluminum.

2. An internal combustion engine valve subjected in use at elevated temperatures to the destructive action of fluctuating atmospheres of combusted fuels under oxidizing, neutral and reducing conditions and containing a corrosive material taken from the group consisting of lead, lead oxide, lead sulfide, lead sulfate and lead bromide, said valve being comprised of an age-hardened, silicon-containing, nickel-base alloy possessing corrosion resistance to the lead oxide test and consisting essentially of about 15% to 17% chromium, about 2.75% to 3.35% titanium, about 1.75% to 2.5% manganese, silicon up to about 0.15%, up to about 0.10% carbon, iron up

7 to about 8%, up to not more than 0.10% aluminum, and the balance nickel.

3. A heat-resisting internal combustion engine valve part having substantial resistance at elevated temperatures to the destructive action of fluctuating, corrosive, lead-containing atmospheres under oxidizing, neutral and reducing conditions, said heat-resisting valve part being comprised of an age-hardened alloy possessing corrosion resistance to the lead oxide test and 10 consisting essentially of about 15% to 17% chromium, about 2.75% to 3.35% titanium, silicon up to about 0.05% to 2.5% manganese, iron up to about 0.15%, up to about 0.10% carbon, iron up to about 8%, and the balance nickel, said alloy 15 being substantially devoid of aluminum.

4. A heat-resisting alloy suitable for internal combustion engine valves and valve parts and having substantial resistance at elevated temperatures to the destructive action of fluctuating atmospheres of corrosive lead-containing fuels under oxidizing, neutral and reducing conditions,

said heat-resisting alloy possessing corrosion resistance to the lead oxide test and consisting essentially of about 15% to 17% chromium, about 2.75% to 3.35% titanium, about 0.05% to 2.5% manganese, silicon up to about 0.15%, up to about 0.10% carbon, iron up to about 8%, up to not more than 0.10% aluminum, and the balance nickel.

CLARENCE GEORGE BIEBER.  
WALTER FRANKLIN SUMPTER.

## References Cited in the file of this patent

## UNITED STATES PATENTS

| Number    | Name           | Date          |
|-----------|----------------|---------------|
| 2,048,167 | Pilling et al. | July 21, 1936 |
| 2,515,185 | Bieber et al.  | July 18, 1950 |

## FOREIGN PATENTS

| Number  | Country       | Date          |
|---------|---------------|---------------|
| 328,362 | Great Britain | May 8, 1930   |
| 583,845 | Great Britain | Jan. 1, 1947  |
| 626,204 | Great Britain | July 12, 1949 |